

July 31, 1945.

H. B. DE VORE

2,380,505

## METHOD OF MANUFACTURING MOSAIC ELECTRODES

Filed June 26, 1941



Fig. 1



Fig. 2



Fig. 3

INVENTOR

By

BY  
*Charles M. Clark*  
ATTORNEY

## UNITED STATES PATENT OFFICE

2,380,505

## METHOD OF MANUFACTURING MOSAIC ELECTRODES

Henry B. De Vore, Newark, N. J., assignor to Radio Corporation of America, a corporation of Delaware

Application June 26, 1941, Serial No. 399,841

3 Claims. (Cl. 204—12)

My invention relates to television transmitting tubes and more particularly to electrode structure of the so-called mosaic type for use in such tubes.

It is known that a sensitive television transmitting or pickup tube of the type in which the picture is transmitted by scanning a mosaic-like target with an electron beam can be made by employing a two-sided mosaic target. In this type of tube an optical image is formed on a photocathode to liberate electrons as an electron image which is focused on one side or face of the target, forming an equivalent electrostatic charge image thereon. Alternatively the charge image may be formed by focusing the optical image on the mosaic directly, provided the side of the mosaic receiving the light image is photo-emissive. This charge image is transmitted conductively through the target to the opposite surface which is scanned by an electron beam. The discharge of elemental areas of the target by the scanning process generates a television signal on a signal electrode which is in capacitive relationship with the elements of the mosaic target.

The conductivity through the target over each elemental picture area must be relatively high to permit the rapid transfer of the charge from the picture side to the scanned side of the target. The conductivity along the target from one elemental area to another must be very low in order to have good resolution in the transmitted picture. In addition, the capacity between each element and the signal plate or electrode should be high in order that a large charge may be stored for the production of a large picture signal. Furthermore, the side of the target on which the electron image is focused should have a high secondary electron emission ratio in order that the intensity of the electrostatic charge image may be increased by secondary electron emission from the target. It has been customary to provide such targets by electrically insulating a wire mesh screen and filling the interstices of the insulated screen with metal plugs. It is very difficult to form such a structure having over 100,000 electrically discrete highly insulated metal plugs, and in addition, even though such electrodes are prepared with exceptional care it has been found that in operation a spurious signal not representative of the electron or optical image is produced which is probably due to electrical and mechanical nonuniformities over the target surface.

It is an object of my invention to provide a television transmitting tube having higher sensitivity with lower distortion than tubes constructed here-

tofore. It is a further object to provide new and novel mosaic electrode structure for use in such tubes as well as a method of manufacturing such structure.

5 In accordance with my invention I provide a tube having a mosaic-type electrode wherein the electrode comprises a sheet of porous insulating material impregnated with metallic particles and wherein the electrical resistance through the sheet normal to its surface is relatively low in comparison with the electrical resistance measured laterally of the porous insulating sheet. Inasmuch as the sheet does not include an electrically conducting foundation, I provide an electron permeable electrode closely adjacent and uniformly spaced from the porous insulating sheet containing the metal particles impregnated therein. Further in accordance with my invention I provide a method of manufacturing a mosaic-type electrode wherein a thin porous sheet of insulating material is coated over various areas thereof or impregnated with a metal salt which is then fused and reduced or converted into the metal which is one of the components of the salt. 10 15 20 25 30 35 40 45 50 55 60 65 70 75 80 85 90 95

Alternately my method of manufacture may include a reduction or conversion of the metallic salt without the fusing step. These and other objects, features and advantages of my invention will become apparent when taken in connection with the following description and the accompanying drawing in which:

Figure 1 is a longitudinal cross-sectional view of a television transmitting tube incorporating my invention;

Figure 2 is a view of a portion of the electrode structure shown in Figure 1, and

Figure 3 is a greatly enlarged sectional view of a portion of the electrode target structure shown in Figures 1 and 2.

While I will particularly describe a type of transmitting tube incorporating means to form an electrostatic image on a mosaic electrode by directing electrons thereon and intensifying the electrostatic image by secondary electron emission, it will be appreciated that my invention is not limited to the use of my new and improved electrode structure in such a tube, but that it may be used to equal advantage in arrangements wherein the electrostatic image is formed on the mosaic electrode directly by the emission of photo-electrons under the influence of the optical image of which an image replica is to be transmitted.

Referring to Figure 1 which shows the former type of tube referred to above, I provide a tube comprising an evacuated envelope enclosing at

one end an electron gun or beam forming structure 2 and at the opposite end a semitransparent photocathode 3 of the conventional type with a target or mosaic electrode 4 intermediate the structure 2 and photocathode positioned to be scanned on one side by an electron beam and to have an electrostatic image formed on the opposite side. This electrostatic image may be formed on the rear surface of the target 4 by projecting light, such as represented by the object arrow 5, through the lens 6 upon the photocathode 3 to liberate electrons therefrom, and focusing the electrons to form an electron image on the target by well-known electron lens structures, or the light may be projected directly upon the rear surface of the target in accordance with the latter method referred to above.

The electron beam forming assembly 2 is preferably of the low velocity electron beam generating type, as described by Albert Rose in his U. S. Patent 2,213,174, or in my copending application, Serial No. 353,792, filed Aug. 23, 1940, and comprises a cathode 7 from which electrons may be drawn, control electrode 8 connected to the usual biasing battery and an anode 9 provided with a beam limiting aperture through which electrons may be directed toward the target 4, the anode 9 being maintained at a positive potential with respect to the cathode by a battery or potential source 10.

Intermediate the electron gun 2 and the target 4 I provide a pair of deflection plates 11 which are curved to produce a uniformly increasing and decreasing electrostatic deflection field, a pair of shield plates 12-13, one on either side of the deflection plates 11 having slots for the passage of the electron beam, and a conductive wall coating 14. The plates 11 are connected to a source of deflection potential and to the shield plates 12-13 and coating 14, through a center-tapped resistance of 1 to 10 megohms. To produce the desired deflection and focus of the electron beam I provide means to wholly immerse the deflection plates in a uniform magnetic field which is preferably generated by a magnetic coil 15 of larger diameter than the envelope 1 extending over and beyond the space between the electron gun 2 and target 4. In the modification of my invention shown in Figure 1 the coil 15 preferably extends beyond the photocathode 3 to focus the electron beam from the photocathode upon the rear surface of the target 4, although an auxiliary short coil may be used between the photocathode 3 and target 4, or a known electrostatic electron image forming structure may be used. The electrons from the photocathode 3 are accelerated over a portion of their path by an electrostatic field such as generated by the wall coating 16 operated at a positive potential with respect to the cathode 7 by a battery or other potential source 17.

Deflection of the electron beam in a direction normal to that produced by the plates 11 is accomplished by a pair of deflection coils 18. This deflection is preferably the frame or vertical deflection, since in standard television systems the frame deflection is of lower frequency than the horizontal line deflection, the coils 18 therefore being operated at the lower of the two frequencies. The deflection coil 18 may, of course, be replaced by a second pair of deflection plates or the deflection plates may be replaced by a second pair of deflection coils, and in fact, any other type of electron gun and associated deflection

structure capable of resolving an electron beam may be used in the place of those described.

In accordance with my invention the target comprises a very thin imperforate target sheet 19 of homogeneous electrically nonconducting material supported as shown in Figure 1 in a plane normal to the longitudinal axis of the envelope 1 and consequently normal to the projected electron beam. Closely associated with the target sheet 19 of electrically nonconducting material and preferably adjacent the rear surface of the sheet I provide a signal electrode 20 coextensive with and very closely spaced with respect to the rear surface of the sheet 19. The signal electrode 20 is electron permeable such as a wire mesh screen and is connected to the input circuit of a translating device 21 and through an output impedance 22 to the cathode 7 either directly or through a portion of the potential source 10. Further in accordance with my invention, and as best shown in Figures 2 and 3, I provide the target sheet 19 of porous material capable of absorbing the metal or metal salt with which I impregnate the sheet during the manufacturing process to form individual mutually separated particles 23 which are preferably highly insulated one from another. For the sheet 19 of porous nonconducting material I prefer to utilize a sheet of aluminum oxide which is formed by oxidation of a thin sheet of aluminum by an electrolytic method such as disclosed in my copending application, Serial No. 388,237, filed April 12, 1941. The method therein disclosed comprises the complete oxidation of a metal sheet by gradual immersion of the sheet in an electrolytic bath of such nature that the bath has the property of dissolving a portion of the formed oxide and wherein the level of the bath is varied during the immersion of the sheet, and the electrolytic current density is maintained substantially constant. As I have pointed out in the said application, the electrolytic bath may be a solution including sulphuric or oxalic acids and the thickness of the formed oxide may be increased indefinitely if proper precautions are taken with respect to cooling the metal sheet and the formed oxide, although I prefer to use for the present application an oxide sheet having a thickness between .001 and .002". I have found that aluminum oxide sheets formed in accordance with my prior manufacturing method are sufficiently thin, have high electrical resistance and are sufficiently porous. The pores of an oxide sheet made as described above extend normal to the surface of the sheet and it is for this reason that such an oxide sheet is ideally suited for forming a mosaic electrode in accordance with my teaching. As a result of this preferential alignment of the pores, the conductivity of my completed electrode is low laterally of the sheet but sufficiently high normal to the surface for satisfactory use as a mosaic.

In accordance with my invention I fill the pores of the formed metal oxide sheet with electrically conductive material so that the resistance from one surface of the sheet to the other is relatively low in the region of the filled pores. Prior to filling the pores with conductive material I thoroughly dry the formed oxide sheet following the electrolytic formation process. I then deposit on one surface of the sheet a metal compound such as a metal salt which may be easily reduced to the metal. For example, particles of silver nitrate may be applied at random to one surface of the sheet by a dusting or spraying operation.

ation. The silver nitrate is preferably in solid form rather than in solution, although for certain purposes a solution may be used. If, however, the solid silver nitrate is applied to the sheet such as by dusting or spraying, the sheet is then heated at a relatively low temperature (approximately 220° C.) until the particles of silver nitrate fuse and soak into the pores of the sheet. Depending on the quantity of silver nitrate used and the temperature, the time of diffusion or soaking into the sheet may vary from 1 minute to 10 minutes. The thin metal oxide sheet carrying the diffused silver nitrate is then placed in an oven which is maintained at a temperature of 500 to 600° C. for a sufficient period of time to reduce the silver nitrate to metallic silver. This baking step and resultant reduction of the metal salt to the metal requires only a short time, such as from 5 to 10 seconds. In the event that a solution of a metal compound or salt is used, the intermediate step of fusing the material and allowing the fused salt to soak into the porous sheet may be unnecessary, in which case the sheet may be placed directly in the oven for the purpose of reducing the metal salt to the desired metal. I have disclosed the use of silver nitrate as an example of reducible metal salt because silver is one of the most suitable metals for use in combination with a mosaic electrode of the photosensitive type. Thus I do not wish to limit myself in practicing my invention to the use of a salt reducible to silver inasmuch as other metal salts such as gold chloride or platinum chloride or other compounds can conveniently be reduced to the free metal. These compounds may be applied by spraying with an oil suspension of the type used to form metal coatings on glass.

Following the preparation and filling of the pores of the insulating sheet with metal, the same may be sealed within the television transmitting device, such as the tube shown in Figure 1, in close proximity to an electron or light permeable electrode such as a wire mesh screen to serve as the signal electrode 20 shown in Figure 1. However, to obtain more uniform spacing between the signal electrode and the thin metal oxide sheet these parts may be assembled prior to introduction within the tube, as shown in Figure 2, by supporting the metal oxide sheet and the signal electrode in a frame 24 separated by a border of insulating material such as a cut-out sheet of mica 25 so that the electrode is exposed on one side of the assembly, and the oxide sheet containing the metal particles formed by the reduction of the metallic salt is exposed on the opposite side of the assembly.

As indicated above, the assembly of the oxide sheet and associated signal electrode is assembled in the tube with the exposed surface of the oxide sheet facing the electron beam forming structure with the opposite side facing the signal electrode and the photocathode 3 or the lens system 6 through which the light forming the optical image is directed. For use in applications where an electron image is directed and focused upon the mosaic electrode it is desirable to treat the surface impinged by the electrons of the image to render it highly secondary electron emissive. Such treatment may comprise depositing a metal of low work function such as caesium directly on the exposed surfaces of the metal particles 23. However, if the electrode is to be of the photo-

emissive type, the metal particles may be oxidized and treated with an alkali metal as well known in the art. Since a photo-emissive surface is likewise highly secondary electron emissive, a single treatment to render the electrode electron emissive under radiant energy such as electron energy or light may be used. Such processing to render electrodes of the type described highly electron emissive are well known in the art.

While I have described an improved type of mosaic electrode and a method of manufacture, it will be appreciated that I am not limited to the materials herein set forth or the particular steps or sequence of the method of manufacture, but that many variations may be made in both the structure and method whereby the structure is obtained without departing from the scope of the appended claims.

I claim:

1. The method of making a two-sided mosaic electrode for television tubes comprising substantially completely oxidizing a thin sheet of aluminum by electrolytic action in a bath capable of dissolving a portion of the formed oxide and continuing said action until sufficient oxide is dissolved to form pores extending from one outer surface of the sheet to the other, placing silver nitrate on one surface of the porous sheet of oxide, heating said sheet to the melting point of said nitrate, continuing the heating until said nitrate is drawn away from said outer surface and into said pores, and heating the impregnated oxide sheet until the silver nitrate is reduced and all the silver is held entirely within said pores and extends from one side of the mosaic to the other with said outer surfaces free thereof.

2. The method of making a two-sided mosaic electrode for television tubes comprising substantially completely oxidizing a thin sheet of aluminum by electrolytic action in a bath capable of dissolving a portion of the oxide and dissolving sufficient aluminum oxide to form pores extending from one outer surface of the sheet to the other, placing a metal compound on one surface of the porous sheet of oxide, heating said sheet to the melting point of said compound, continuing the heating until said compound is drawn away from said outer surface and into said pores, and heating the impregnated oxide sheet until said compound is reduced and the metal is held entirely within said pores and extends from one side of the mosaic to the other with said outer surfaces free thereof.

3. The method of making a two-sided mosaic electrode for television tubes comprising immersing a thin sheet of aluminum in an electrolyte capable of slowly dissolving aluminum oxide, substantially completely transforming said sheet by electrolysis to aluminum oxide, continuing the immersion of said sheet until sufficient aluminum oxide is dissolved to form pores extending entirely through said sheet at a multiplicity of points, removing the sheet from the electrolyte, filling the pores thereof with a metal salt reducible at moderate temperature, and heating the impregnated sheet until the salt in said pores is reduced and held entirely within said pores and extends from one side of the mosaic to the other and the outer surfaces are free thereof.

HENRY B. DE VORE.